

# United States Patent [19]

Hirakawa et al.

[11] Patent Number: 4,582,747

[45] Date of Patent: Apr. 15, 1986

[54] DUST-PROOF FABRIC

[75] Inventors: Tadashi Hirakawa, Kusatsu; Mamoru Tsumoto, Ibaraki, both of Japan

[73] Assignee: Teijin Limited, Osaka, Japan

[21] Appl. No.: 701,557

[22] Filed: Feb. 14, 1985

[30] Foreign Application Priority Data

Feb. 16, 1984 [JP] Japan ..... 59-26132  
Jun. 7, 1984 [JP] Japan ..... 59-115391

[51] Int. Cl. 4 D03D 15/00

[52] U.S. Cl. 428/229; 55/528;  
55/DIG. 43; 55/DIG. 45; 428/311.1;  
428/311.5; 428/315.5; 428/315.7; 428/317.9;  
428/401; 428/922; 428/374

[58] Field of Search 428/229, 311.1, 311.5,  
428/315.5, 315.7, 317.9, 922; 55/DIG. 43,  
DIG. 45, 528

[56] References Cited

U.S. PATENT DOCUMENTS

3,986,530 10/1976 Maekawa ..... 55/DIG. 43

|           |         |                     |           |
|-----------|---------|---------------------|-----------|
| 4,025,679 | 5/1977  | Denny .....         | 55/528    |
| 4,499,139 | 2/1985  | Schortmann .....    | 428/315.5 |
| 4,520,066 | 5/1985  | Athey .....         | 428/311.5 |
| 4,539,255 | 9/1985  | Sato et al. .....   | 428/315.5 |
| 4,540,625 | 9/1985  | Sherwood .....      | 428/311.5 |
| 4,547,423 | 10/1985 | Kojima et al. ..... | 428/317.9 |

FOREIGN PATENT DOCUMENTS

104548 6/1985 Japan .

Primary Examiner—James C. Cannon  
Attorney, Agent, or Firm—Burgess, Ryan & Wayne

[57]

ABSTRACT

A dust-proof fabric having an excellent dust-collecting efficiency and dust-preventing property including a plurality of filament yarns having a thickness of 20 to 400 denier and consisting of a plurality of individual filaments having a denier of 3.5 or less. The fabric has a number of pores formed therein and exhibits an air permeability of 0.3 to 10 ml/cm<sup>2</sup>/sec. In the fabric, the proportion of the integrated volume of pores having a size of 43  $\mu$ m or more to the entire integrated volume of all the pores in the fabric is 40% or less.

12 Claims, 3 Drawing Figures







## DUST-PROOF FABRIC

## BACKGROUND OF THE INVENTION

## 1. Field of the Invention

The present invention relates to a dust-proof fabric. More particularly, the present invention relates to a dust-proof fabric useful for preparing dust-proof clothing to be used in clean rooms, for example, industrial clean rooms, biological clean rooms and surgical operation rooms, which are effective for preventing contamination of the human body or specific articles with dust generated from machines and human personnel.

The dust-proof fabric of the present invention generates dusts therefrom in a very reduced amount and can collect dust at a high efficiency. Also, the dust-proof fabric of the present invention exhibits an antistatic property which prevents excess attraction of dust and prevents breakdowns of semiconductor devices.

## 2. Description of the Related Art

It is known that to prevent undesirable generation of dust from clothing of workers or operators in industrial clean rooms and other clean rooms by use of dust-free clothing (inclusive of sterile clothing). The dust-free clothing is produced from woven or knitted fabrics consisting of synthetic filament yarns or nonwoven fabrics consisting of spun bonded continuous filaments. Also, it is known to prevent undesirable adhesion of dust on the dust-free clothing by antistatic treatment applied to the dust-free clothing.

With recent increase of precision, integration, and miniaturization in the semiconductor industry and precision machine industry and in the fields of the bioindustry and medical industry, clean rooms have come into broad use. It is especially required at the present time that the cleanliness of air in a clean room be further increased. For example, in the field of semiconductors, the integration degree in LSI's is being increased to 256 K-bits from 64 K-bits. It is expected that the integration degree will be elevated to 1 M-bit (megabit) or higher in the not too distant future. It is ordinarily considered that the air cleanliness degrees of clean rooms required for these integration degrees are class 1000-100, class 100-10, and class 10 or lower. It also is considered that the size of dust to be removed becomes smaller as the air cleanliness is elevated. Namely, minute dust or bacteria cause defects in products. Hence, the higher the air cleanliness, the more important the prevention of generation of dust. Accordingly, with elevation of the cleanliness of a clean room, enhancement of the dust-preventive effect in dust-free clothing is required.

The largest dust-generating sources in a clean room are the human personnel themselves. The contamination level in the clean room is elevated by dust generated from the personnel. The dust-generating sources of human personnel include (1) the physical bodies, (2) undergarments, and (3) outer dust-free clothing. Generation of dust from the clothing can be greatly reduced by using a filament yarn and periodically cleaning the dust from the clothing. The main sources of dust are therefore the body and undergarments of the personnel. Accordingly, it is necessary that dust generated from the body or undergarments be prevented from being discharged outside.

Therefore, the clothing should be made of dust-proof fabric which prevents discharge of dust outside from the clothing. Of course, it must be excellent in adaptability, durability, and comfort. As means for prevent-

ing discharge of dust, there has been proposed a fabric with a low dust permeability, that is, a high dust-collecting property (high filtering property). Conventional woven and knitted fabrics, however, have a high dust permeability (low dust-collecting efficiency). Certain spun-bond non-woven fabrics have low dust permeability, but they also have a paper-like stiff touch and poor washing resistance.

Recently, as means for reducing the dust permeability of a woven or knitted fabric and preventing discharge of dust, the dust-free clothing has been made from a fabric obtained by resin-coating a woven or knitted fabric of synthetic filaments or a fabric obtained by laminating a film on a woven or knitted fabric of synthetic filaments. According to this technique, the fabric is coated, e.g., with a water-proof moisture-permeable resin such as a polyurethane resin to reduce the air permeability while maintaining a certain moisture permeability. Clothing of this type does not allow permeation of air, and resists, permeation of dust. However, such clothing is defective in various points. For example, since the moisture permeability and air permeability are poor, the clothing becomes uncomfortable on wearing. A resin-coated (or laminated) fabric is also ordinarily poor in durability, washing resistance, and abrasion resistance. Clothing to be used in a clean room is frequently subjected to dry cleaning, but a water-proof moisture-permeable resin is ordinarily poor in dry cleaning resistance. In short, a fabric for dust-free clothing, which is satisfactory in dust-collecting efficiency, wearing properties (moisture permeability and air permeability), wearing durability, washing resistance, abrasion resistance and antistatic property has not been developed.

## SUMMARY OF THE INVENTION

An object of the present invention is to provide a dust-proof fabric having an enhanced dust-preventing property useful for producing dust-free clothing for clean rooms having a highly enhanced air cleanliness.

The above-mentioned object can be attained by the dust-proof fabric of the present invention, which includes a plurality of filament yarns having a denier of from 20 to 400 and consisting of a plurality of individual filaments having a denier of 3.5 or less. The fabric has a number of pores formed therein and exhibits an air permeability of from 0.3 to 10 ml/cm<sup>2</sup>/sec. In the fabric, the integrated volume of the pores having a size of 43  $\mu$ m or more corresponds to 40% or less of the entire integrated volume of all the pores.

The dust-proof fabric of the present invention is preferably in the form of a woven fabric composed of a plurality of warp and wefts consisting of the filament yarns. Also, it is preferable that the warp and/or wefts contain electrically conductive filament yarns having an electric resistivity of  $10^{10} \Omega/\text{cm}$  or less and arranged at intervals of from 3 mm to 50 mm.

## BRIEF DESCRIPTION OF THE DRAWINGS

FIGS. 1, 2, and 3 are graphs showing the relationship between the size in  $\mu$ m of pores in the fabrics of the present invention and comparative fabrics and the volume fraction of the pores having a size in percent based on the entire integrated volume of all the pores in each fabric.

## DESCRIPTION OF THE PREFERRED EMBODIMENTS

With a view to developing a fabric for dust-free clothing satisfactory in all of the foregoing properties, the inventors made extensive research on the structure of such a fabric, practical properties such as the dust-collecting efficiency and durability characteristics, the antistatic property, and the dust-preventive property of dust-free clothing on actual wear. As a result, they obtained a novel finding about the mechanism of generation of dusts and invented a fabric for anti-static dust-free clothing having a novel structure. It has been considered that generation of dust from human personnel would be reduced in dust-free clothing composed of a fabric having a low dust permeability. Improvements of fabrics for dust-free clothing have been made based on this idea. However, there has been no knowledge about the relation between the dust permeability of the fabric for a dust-free clothing and generation of dust in the dust-free clothing on actual wear. It has not been proved whether the above idea is correct. Moreover, the relation between the structure of a fabric for dust-free clothing and the dust-collecting efficiency has not been investigated in detail. It has not been clarified what structure of a dust-proof fabric would be effective for increasing the dust-collecting efficiency.

The inventors produced, on an experimental basis, various types of dust-proof clothing from various types of dust-proof fabrics differing in dust permeability and air permeability and checked the amount of dust generated from the clothing when personnel wearing the clothing worked. As a result, they found surprisingly, that, in case of dust-free clothing composed of a resin-coated or laminated fabric having no substantial dust permeability, the amount of generated dust is large and when the dust permeability or air permeability is within a certain range, the amount of generated dust is reduced to a minimum. More specifically, in case of a fabric having no substantial air permeability, contaminated air having a high dust concentration within dust-free clothing does not permeate the fabric but leaks out from openings of the clothing such as the edge of the sleeves or the neck portions. In contrast, in case of a dust-free clothing composed of a fabric having an appropriate air permeability and a high dust-collecting efficiency, when contaminated air within the space surrounded by the dust-free clothing permeates the fabric, the dust in the contaminated air is collected by the dust-proof fabric. Therefore, it is considered that leakage of contaminated air from openings is reduced, resulting in decreased dust. Namely, reduction of the dust permeability by reducing the air permeability of a fabric is insufficient for drastically reducing dust generated from personnel. It is necessary that the dust permeability be low and appropriate air permeability be given to the fabric. Moreover, since a conventional fabric does not have a sufficient antistatic property, the fabric is readily charged and dust is attracted to the clothing, with the result that generation of dust from the clothing becomes conspicuous or semiconductors are broken by discharges from the charged fabric. Accordingly, it has been considered preferable to impart an antistatic effect in addition to the above-mentioned dust-preventing property.

In the dust-proof fabric of the present invention, the material of the multifilament yarns is not particularly critical. For example, the material of the multifilament

yarns may be selected from polyesters, such as polyethylene terephthalate (PET) and polybutylene terephthalate (PBT); polyamides, for instance, nylon-6, nylon-66, and aromatic polyamides; polyolefins, for example, polyethylene and polypropylene; polyvinyl polymers, for instance, polyvinyl alcohol, polyvinyl chloride, and polyacrylonitrile; rayon; cellulose acetate; silk; and glass. The multifilament yarn may be composed of one of these materials or composed of two or more of these materials. In some case, good chemical resistance is required for dust-free clothing in addition to functions ordinarily required for clothing. Furthermore, it is often required that the dust-free clothing be excellent in durability, washing resistance, and dry cleaning resistance. It is preferred that a material capable of satisfying these requirements in a broad range be used. For example, polyesters such as PET and PBT and polyamides such as nylon-6 and nylon-66 are preferred.

The denier of the individual filaments in the multifilament yarns should be 3.5 or less. The denier of the filament yarns should be in the range of from 20 to 400.

Generally, as described hereinafter, the dust-collecting (filtering) property of the fabric is enhanced with an increase of the ratio of the integrated volume of the pores formed between the individual filaments to the entire integrated volume of all the pores in the fabric. In the case of a filament bundle, that is, a multifilament yarn, the sum of the surface areas of the individual filaments in the bundle having a unit weight increases with a decrease of the denier of the individual filaments. That is, the smaller the denier of the individual filaments in the bundle, the smaller the size of the pores formed between the individual filaments and the larger the integrated volume of the pores formed between the individual filaments in the bundle. Therefore, it is preferable that the individual filaments have a denier as small as possible, that is, of 1.5 denier or less, more preferably about 0.5 or less. The small denier of the individual filaments of 1.5 or less is effective for creating a soft touch of the resultant fabric.

In the case where the integrated volume of the pores formed between the multifilament yarns (bundles) is reduced by increasing the densities of warps and wefts in the fabric, the dust-filtering property of the fabric closely depends on the integrated volume of the pores formed between the individual filaments. In order to enhance the dust-filtering property of the fabric, it is very important to use individual filaments having a denier as small as possible.

An ultrafine multifilament yarn consisting of individual filaments having an extremely smaller denier than that of conventional multifilament yarns is known. Any of the known ultrafine multifilament yarns can be utilized for the present invention. The ultrafine multifilament yarn usable for the present invention can be produced, for example, by a process for producing peelable composite filaments, as disclosed in Japanese Unexamined Patent Publication (Kokai) Nos. 51-70366, 51-130317, 51-58578, and 58-186663 and Japanese Examined Patent Publication (Kokoku) No. 56-16231, by a process for producing islands-in-a-sea type composite filaments, as disclosed in Japanese Examined Patent Publication (Kokoku) Nos. 45-6297, 44-18369, and 58-22126, or by a direct spinning process as disclosed in Japanese Unexamined Patent Publication (Kokai) Nos. 54-30924, 54-73915, 55-1338, and 55-152809. These ultra-fine multifilament yarns can be converted into

woven and knitted fabrics according to known methods.

The cross-sectional profile of the individual filaments is not particularly limited to any specific shape. The individual filaments may have a circular (regular) or a non-circular (irregular) cross-sectional profile such as a triangular, cruciform, hollow, or a star-shaped cross-sectional profile. Of course, a combination of the regular and irregular cross-sectional profiles may be adopted. In order to increase the integrated volume of 10 the pores formed between the individual filaments, use or incorporation of irregular individual filaments having an irregular cross-sectional profile is sometimes advantageous.

The thickness (total denier) of the warps or wefts should be in a range of from 20 to 400. If the total denier of the warps or wefts exceeds 400, the resultant fabric becomes excessively thick and the touch of the fabric is degraded. Moreover, the clearance between the warps or wefts is increased, and the filtering property of the 20 fabric is reduced. When the total denier of the warps or wefts is smaller than 20, the resultant fabric is too thin, and therefore, the strength or durability of the fabric is insufficient and the filtering property of the fabric is unsatisfactory. It is especially preferred that the total 25 denier of the warps or wefts be in a range of from 50 to 250.

The thickness of the fabric is preferably in a range of from 0.05 mm to 0.40 mm. If the thickness of the fabric is larger than 0.40 mm, the filtering property of the 30 fabric increases with increase of the thickness but, sometimes, the resulting dust-free clothing is too heavy and is not comfortable to wear. If the thickness of the fabric is smaller than 0.05 mm, since the fabric is too thin, the strength, the durability, and the filtering property of the resultant fabric are sometimes unsatisfactory.

In connection with the form of the multifilament yarn, a flat yarn or textured bulky yarn may be used. In case of bulky yarns, for instance, a false-twisted yarn or a yarn composed of individual filaments different in the shrinkability, the looseness between the individual filaments is ordinarily larger than that between the filaments in a flat yarn. Accordingly, in a fabric composed of a textured bulky yarn, the integrated volume of the pores formed between the individual filaments is larger than that in a fabric composed of flat yarns and the filtering property of the textured bulky yarn fabric is generally excellent. Therefore, in a woven or knitted fabric composed of separable ultra-fine filaments in which one filamentary component has a higher shrinkability than that of the other filamentary component, the filtering property of the resultant fabric is very excellent because of the very small denier of the peeled-separated filaments, the high bulkiness of the fabric, and a large integrated volume of the pores between the 55 individual ultra-fine filaments.

The dust-proof fabric of the present invention is in the form of a woven fabric selected from, for example, plain weaves, twill weaves and satin weaves, or a knitted fabric selected from, for instance, weft (circular)-knitted fabrics and warp-knitted fabrics. In consideration of mechanical strength, durability, stretchability, rigidity, air-permeability and facility of treatments to be applied to the fabric, the dust-proof fabric of the present invention is preferably in the form of a woven fabric, especially, a plain weave or twill weave.

The pores in the fabric are classified into those of three types, that is, (1) pores (intra-filament pores)

formed on the peripheral surfaces of the individual filaments, (2) pores (inter-filament pores) formed between the individual filaments, and (3) pores (interfilament bundle pores) formed between the filament bundles, that is, the multifilament yarns.

The integrated volume of the pores having a certain size can be measured by a fluid-permeation method, electron microscopic method, or a mercury intrusion method. The mercury intrusion method using a porosimeter is most preferred to precisely and easily determine the volume fraction of the pores having a certain size. In the present invention, the distribution of the volumes fraction of the pores in the fabric is measured by the mercury intrusion method.

The method for measuring the size of the pores will now be briefly described.

Mercury does not substantially wet all substances. Accordingly, mercury does not intrude into pores unless mercury is pressed into the pores. The relation between the pore size (diameter) and the pressure to be applied to mercury is represented by the following equation (1):

$$P \cdot D = -4\sigma \cos \theta \quad (1)$$

wherein P stands for the pressure applied to mercury, D stands for the size (diameter) of the pore, provided the pore is in the form of a cylinder,  $\sigma$  represents the surface tension of mercury, and  $\theta$  represents the contact angle of the specimen to be tested with mercury.

If P,  $\sigma$ , and  $\theta$  are known, the pore size D can be determined from the above equation (1). Moreover, the volume of mercury penetrated into the specimen represents the integrated volume of the pores, and the pore size distribution can be obtained from the pressures applied stepwise to mercury and the volumes of mercury penetrated into the specimen.

The pore size distribution determined with respect to various fabrics according to the mercury intrusion method, are shown in FIGS. 1, 2, and 3 of the accompanying drawings. In each figure, the peaks of the volume fraction appear at the sizes of the pores of 1 to 10  $\mu\text{m}$  and of 20 to 100  $\mu\text{m}$ . It is considered that these peaks correspond to the pores formed between the individual filaments and the pores formed between filament bundles. The integrated volume proportion of the pores having a predetermined size or more or less or a predetermined range of size is represented by a ratio (%) of the integrated volume thereof to the entire integrated volume of all the pores in the fabric.

The volume is expressed in the unit of cubic centimeters per gram of the fabric (ml/g).

When dust passes through a woven or knitted fabric, the larger the size of through pores in the woven or knitted fabric, the higher the permeability of dust through the fabric. Accordingly, in order to reduce permeation of dust, it is first of all important to decrease the size of the through pores. The largest pores in a woven or knitted fabric are the above-mentioned interfilament bundle pores (3) formed between filament bundles. Accordingly, it is important to reduce the size of these pores as much as possible. For this purpose, the pore size distributions in conventional fabrics utilized for making dust-free clothings was measured. As result, it was found that in each of the conventional fabrics, the integrated volume of pores having a size of about 50  $\mu\text{m}$  or more is very large. Based on this fact, the approach taken was to improve the filtering property of conven-

tional fabrics by reducing the size and integrated volume of these large-size pores. As factors having influences on the size and the integrated volume of the inter-filament bundle pores, there are densities of the yarns, the presence or absence of the calender treatment, the conditions of the calender treatment, the form of the yarn used (for example, a flat yarn or a textured bulky yarn), the weaving structure, and the finish density of the fabric. Since the finish density has direct influences on the inter-filament bundle pores, it is preferred that the finish density be increased as much as possible. If this finish density is too low, the inter-filament bundle pores become too large and the filtering property of the fabric is degraded. Ordinarily, the two-dimensional porosity of a woven fabric is represented by the cover factor. However, since this cover factor is not in agreement with the three-dimensional porosity of the fabric, it is difficult to represent the porosity of the fabric by the cover factor. The calender treatment exerts an effect of crushing the pores. Therefore, the calender treatment is a method customarily adopted for reducing the volume of the inter-filament bundle pores in a fabric and imparting a low air permeability to the fabric. This treatment is effective also in the present invention. The volume of the inter-filament bundle pores are variable depending on the weaving structure. Furthermore, when a fabric is greatly shrunk, for example, at the dyeing step, a fabric having a high density can be obtained. In the present invention, a woven or knitted fabric having a small volume of interfilament bundle pores can be obtained by adopting the above-mentioned means singly or in combination.

With respect to the various types of fabrics of the present invention and the conventional fabrics, the relationship between the pore size distribution and the dust-filtering property of the fabric was analyzed. As a result, it was found that a fabric in which the proportion of the integrated volume of pores having an inner size of 43  $\mu\text{m}$  or more is 40% or less, based on the entire integrated volume of all the pores in the fabric, the resultant fabric exhibited an enhanced dust-filtering property. The term "inner size" referred to herein means the pore size determined according to the mercury intrusion method. In the present invention, since  $\theta$  in the above equation (1) is set at 130° and  $\sigma$  is set at 484 dyne/cm, for example, the inner size of 42.6236  $\mu\text{m}$  corresponds to the pressure of 4.2 psia (pounds per square inch absolute) of mercury.

In the case of a fabric in which the integrated volume proportion of pores having an inner size of 40  $\mu\text{m}$  or more exceeds 40%, the dust-filtering property of the fabric is not different from that of the conventional fabrics, and the dust-filtering property of the fabric is prominently improved when the above-mentioned integrated volume proportion is 40% or less. The dust-filtering property is more conspicuously improved when the above-mentioned integrated volume proportion is 25% or less. This effect is due to the fact that the integrated volume of the inter-filament bundle pores is reduced and the integrated volume of inter-filament pores providing a high dust-filtering effect is increased. Reduction of the integrated volume of the inter-filament bundle pores results in prevention of leakage of dust, and increase of the inter-filament pore results in increase of the dust-filtering efficiency of the fabric. A fabric having a very high dust-filtering property and an appropriate air permeability can be obtained only when the integrated volume of the interfilament bundle pores

is reduced and the integrated volume of the inter-filament pores is much increased. In the present invention, the structural requirement to be satisfied for obtaining a fabric having a most highly improved dust-filtering property and an appropriate air permeability is that in the pore size distribution, the integrated volume proportion of pores having an inner size of 0.1 to 10  $\mu\text{m}$  is 28% or more and the integrated volume proportion of pores having an inner size of 43  $\mu\text{m}$  or more is 40% or less based on the entire integrated volume of all the pores in the fabric. In this fabric, as the integrated volume proportion of pores having an inner size of 0.1 to 10  $\mu\text{m}$  is much larger than 28%, and the integrated volume proportion of pores having an inner diameter of 43  $\mu\text{m}$  or more is much less than 40%, the dust-filtering property of the fabric is increased. Especially, a fabric having a structure in which the integrated volume proportion of pores having an inner size of 0.1 to 10  $\mu\text{m}$  is larger than about 40% and the integrated volume proportion of pores having an inner diameter of 43  $\mu\text{m}$  or more is about 10% or less has an appropriate air permeability and a very high dust-filtering property and is most preferred as the fabric useful for making dust-free clothing.

It is easy to obtain a fabric in which permeation of dust is completely prevented. This can be accomplished by depriving the fabric of the air permeability. If permeation of air through the fabric is not allowed, dust which is larger than molecules constituting air should not be allowed to pass through the fabric. However, when dust-free clothing is worn over an undergarment generating large quantities of dust and the personnel works in this state, if the number of dust particles having a size of not less than 0.3  $\mu\text{m}$  is measured, the value of the number of dust particles in dust-free clothing made of a fabric having no substantial air permeability is not close to zero but is larger than the number of dust particles generated in dust-free clothing made from a fabric having air permeability. Even if dust-free clothing made of a fabric having no air permeability or having no substantial air permeability is worn, large quantities of dust are actually generated. With a view to clarifying the cause of this phenomenon, generation of dust was investigated while completely sealing the sleeve edges and neck portion of dust-free clothing made of a fabric having no substantial air permeability. It was found that generation of dust was drastically reduced. Accordingly, it was confirmed that in case of dust-free clothing of this type, since the fabric has no air permeability, entry and exit of air by the motion of the personnel are performed only through the openings in the sleeve edges and neck portion of the clothing and contaminated air is discharged directly from these openings. Accordingly, it is evident that the fabric for dust-free clothing should have appropriate air permeability. By the term "no substantial air permeability", it is meant that the fabric has only a very small air permeability. An air permeability of about 0.2 to about 0.3 cc/cm<sup>2</sup>/sec or less as determined according to the Frazier method of JIS L-1079 is meant.

In a woven or knitted fabric, if the integrated volume of the inter-filament bundle pores is large, and therefore air permeation quantity is too large, in order to improve the dust-filtering property it is ordinarily preferred that the integrated volume of the interfilament bundle pores be reduced to an appropriate level. On the other hand, if the air permeability of a woven or knitted fabric is too low, the moisture permeation becomes insufficient and an uncomfortable feeling is given to a wearer. It is said

that in order to moderate the uncomfortable feeling on wearing, it is necessary that the moisture permeability of a woven or knitted fabric be at least about 4000 g/m<sup>2</sup>/24 hours. In order to impart the moisture permeability of this level to the fabric, it is necessary that air permeability of at least about 0.3 cc/cm<sup>2</sup>/sec, preferably, at least 0.4 cc/cm<sup>2</sup>/sec should be given to the fabric. If the air permeability exceeds 10 cc/cm<sup>2</sup>/sec, the integrated volume proportion of the inter-filament bundle pores becomes too large and the dust-filtering property is reduced. Accordingly, it is indispensable that the air permeability of the fabric should not be higher than 10 cc/cm<sup>2</sup>/sec.

In the fabric of the present invention, it is preferable that electrically conductive multi- or mono-filament yarns having an electric resistivity of 10<sup>10</sup> Ω/cm or less, preferably 10<sup>9</sup> Ω/cm or less, be incorporated into warps and/or a wefts at intervals in a range of from 3 mm to 50 mm. It is preferred that the diameter of the electrically conductive filament yarns be less than 100 μm, more preferably 60 μm or less. The electric resistivity referred to herein is the value measured by fixing both the ends of the filament yarn to aluminum foil by using an electrically conductive paste to form electrodes and applying a voltage of 100 V between the electrodes at a testing length of the yarn of 2 cm. Any of the electrically conductive filament yarns can be used in the present invention irrespective of the preparation process therefor, so far as the electric resistivity of the yarn is 10<sup>10</sup> Ω/cm or less. More specifically, yarns of metal fibers, carbon fibers, and organic electroconductive fibers may be used in the present invention. The organic electroconductive fibers may be selected from products formed by coating the surfaces of synthetic fibers with carbon black or metal powder together with a resin (see Japanese Examined Patent Publication (Kokoku) No. 46-23799), composite fibers including a polymer containing carbon black or metal powder as one component (see Japanese Unexamined Patent Publication (Kokai) No. 48-48715), fibers having a metal complex formed therein by diffusion of a metal ion and fibers containing cuprous iodide in the interior thereof (see Japanese Unexamined Patent Publication (Kokai) No. 57-35004). The electrically conductive filament yarns were inserted into warps and/or a wefts at intervals in a range of from 3 mm to 50 mm in the fabric of the present invention. If the distance between the conductive yarns is larger than 50 mm, the resultant antistatic effect is sometimes unsatisfactory. If the distance is less than 3 mm, the resultant antistatic effect is saturated. In the present invention, fabric having or not having the electrically conductive filament yarns incorporated therein may be further treated with an antistatic agent, or antistatic synthetic filament yarns may be used as warps and/or wefts.

The electrostatic charge density of the antistatic fabric of the present invention is usually 7 μC/m<sup>2</sup> or less.

An increase of the denier of individual filaments is effective as means for increasing the integrated volume of inter-filament pores. However, in order to increase this volume, it is necessary not only to reduce the denier of the individual filaments but also to make contrivances on the interior structure of the filament bundle. In the case where the individual filaments are gathered substantially in parallel to one another in the filament bundle as in the case of a flat yarn, since the individual filaments are close to one another along the longitudinal direction, the volume of the pores between the individual

filaments, that is, of the inter-filaments pores should inevitably be reduced. Even though the above-mentioned volume may be increased by reducing the denier of the individual filaments, this increase is limited in the case of a flat yarn. Accordingly, in the case of a fabric composed of flat yarns, even if the integrated volume of pores having an inner size of 43 μm or more is reduced as compared with this volume in the conventional fabrics and the denier of the individual filaments is reduced, the enhancement of the filtering capacity of the fabric is limited. Also, in order to further enhance the dust-filtering property of the fabric, it is necessary to drastically reduce the air permeability thereof. In order to enhance the dust-filtering property of the fabric, it is preferred that the integrated volume of the pores formed between the filament bundles be reduced, the denier of the individual filaments be reduced, and the integrated volume of pores having an inner size in a range of from 1 μm to 10 μm be further increased, so that dust can be filtered through the pores formed between the individual filaments, that is, the inter-filament pores. A fabric having a large integrated volume of pores having the above-mentioned inner size can be prepared, for example, according to the following methods.

(1) A fabric is produced by weaving crimped multifilament yarns (for example, false-twisted yarns) consisting of individual filaments having a denier of about 1 used as warps and wefts. In order to reduce the integrated volume of the inter-filament bundle, weaving procedures are carried out so that the densities of the warps and wefts are as high as possible. The obtained fabric is then scoured and dyed according to customary procedures and is calendered by a compressing hot roll. The temperature of the hot roll is about 150° C. to about 220° C. and the pressure is about 10 to about 80 kg/cm<sup>2</sup>. If necessary, the fabric is subjected to cam-fit processing to soften the touch of the woven fabric. In this woven fabric, the integrated volume proportion of pores having an inner size of 43 μm or more is lower than that of the conventional fabrics, and the integrated volume proportion of pores having an inner size in a range of from 1 μm to 10 μm is higher than that of the conventional fabrics.

(2) A fabric is obtained by weaving by using, as warps, polyester multi-filament yarns consisting of individual filaments having a denier of 1 or less and, as wefts, separable hollow composite filament yarns in which a polyester filamentary component and a polyamide filamentary component are arranged in the multi-annular configuration adjacent to each other and they are extended in the longitudinal direction of the yarn to form a tubular structure as a whole. The denier of the respective components of the hollow composite filament yarns is in a range of from 0.001 to 0.8. This fabric is scoured and dyed according to customary procedures. The fabric is subjected to a splitting treatment. The splitting treatment is accomplished, for example, by immersing the fabric in an aqueous emulsion of phenylphenol compounds, benzyl alcohol, chlorobenzene compounds, alkylbenzene compounds, or diphenyl compounds at a temperature of about 10° C. to about 40° C. Then, the fabric is calendered by a pressing hot roll. The temperature of the pressing hot roll is about 130° C. to about 180° C., and the pressure is about 10 to about 80 kg/cm<sup>2</sup>. Since the nylon-6 filamentary components are greatly shrunk at the splitting treatment and the dyeing step, the density of the fabric is greatly increased.

creased and the denier of the individual filaments is remarkably reduced by splitting. A great difference of the length is produced between the polyester filamentary component and the nylon-6 filamentary component. Accordingly, a fabric in which the integrated volume of the inter-filament bundle pores is very small and the integrated volume of the inter-filament pores is very large is obtained.

(3) In the above-mentioned method (2), the separable composite filament yarn is used only as wefts, but it is preferred that this separable composite filament yarns be used as both the warps and the wefts. The splitting treatments are conducted in the same manner as in method (2). The structure of the obtained woven fabric is preferable to the structure of the woven fabric obtained according to method (2).

(4) The above-mentioned separable composite filament yarn mentioned in method (2) is twisted at a twist number of 1500 to 3500 T/M at room temperature to partially split the peripheral portions of the composite filament yarns contacting each other. Then, weaving and processing are carried out as in methods (2) or (3). Since partial splitting is effected before weaving, the splitting can be easily done by the splitting treatment conducted after weaving, and the final splitting degree is higher than in method (2) or (3).

(5) The composite filament yarn used in method (2) is subjected to a compressed air jetting treatment (for example, under a compressed air pressure of 4 kg/cm<sup>2</sup> at room temperature at an overfeed rate of 10%), and the resulting interlaced yarns are woven and processed as in method (2) or (3) (see Japanese Patent Application No. 58-189997).

(6) A woven fabric prepared according to method (2) or (3) is subjected to a wet heat treatment at a temperature of 50°C. or more before the splitting treatment, and the fabric is then subjected to the splitting treatment.

(7) The composite filament yarns described in method (2) are subjected to a texturing procedure, for example, are false-twisted at a heater temperature of about 180°C. The textured yarns are connected to a woven fabric. The fabric is finished in the same manner as that described in method (2).

The following effects can be attained by the present invention.

(1) Since the woven or knitted fabric of the present invention is composed of continuous multifilament yarns, generation of dust from the fabric per se is small.

(2) Since the fabric of the present invention has a dense structure in which the integrated volume of large pores or pores having a low dust-collecting efficiency and allowing permeation of dusts is small and the integrated volume of small pores having a high dust-collecting efficiency is large, the dust-collecting efficiency of the fabric is much higher than that of the conventional fabrics.

(3) Since the fabric of the present invention has an appropriate air permeability and a high dust-collecting efficiency, (a) the dust-preventing effect of the resulting dust-free clothing is high and (b) no uncomfortable feeling is caused on wearing.

(4) The fabric of the present invention is soft and has a soft touch, and dust-free clothing made of this fabric has excellent comfort and touch.

(5) Since the fabric of the present invention is not coated or laminated with a resin, the fabric is excellent in the washing resistance and the abrasion resistance,

gives no uncomfortable feeling on wearing and has a soft touch, and excellent comfort and touch to the skin.

(6) When electrically conductive filament yarns are incorporated, the dust-proof fabric of the present invention exhibits not only a high dust-filtering property but also a high antistatic effect.

(7) The fabric of the present invention can be utilized for making dust-free clothing, sterile clothing, dust-preventive clothing, and clothing to be used in a clean room, such as hoods, head caps, hats, shoes, socks, boots, mask, gloves, undergarments, inner suits, and aprons.

The present invention will now be described in detail with reference to the following examples. Incidentally, in the present invention, the properties of the fabrics are evaluated according to the following methods.

(1) Integrated volume of pores in relation to the size of the pores

A mercury intrusion porosimeter (trademark: Micromeritics Auto Pore 9200, made by Shimazu Seisakusho K. K.) was used as the measurement device. The mercury pressure was in a range of from 1.9 to 60,000 psia (corresponding to the size of pores of 94 to 0.003 μm). Within the above-mentioned range, 43 levels of the pressure were set. The weight of the specimen was 3 g. It was presumed that the contact angle of mercury was 130° and the surface tension of mercury was 484 dyne/cm. The pore size was calculated according to the equation (1). The entire integrated volume of all the pores in a fabric refers to the sum of the volumes of pores having an inner size of 0.003 μm (corresponding to a mercury pressure of about 60,000 psia) or more in the fabric. The entire integrated volume of all the pores was expressed in the unit of volume (ml) per gram of the fabric (ml/g). The integrated volume proportion of the pores having an inner size of 43 μm or more was represented in percent thereof based on the entire integrated volume of all the pores in the fabric. The integrated volume proportion of pores having an inner size in a range of from 0.1 μm to 10 μm was determined by subtracting the integrated volume of pores having an inner size of 9.8585 μm or more from the integrated volume of pores having an inner size of 0.0937 μm or more, and expressed in percent based on the entire integrated volume of all the pores in the fabric. In each volume fraction diagram in FIGS. 1 through 3, the size of pores means an average pore size. The volume fraction refers to the integrated volume of pores having sizes corresponding to mercury pressures in the range between two adjacent two levels from which the average pore size was calculated.

(2) Dust-collecting efficiency (η) of fabric

The dust-collecting efficiency of the fabric was evaluated in an air-conditioned room where the fluctuation in concentration and particles size distribution of dust in air was small. A fabric specimen was attached air-tight to a stainless steel funnel having an effective diameter of 18 cm. A conduit connected to the funnel was connected to a dust counter (Trademark: Model 4100 made by Dan Kagaku K. K.) through a plastic tube. The dust counter was actuated, the sample air suction rate was adjusted to 0.3 liter/min (or 1/min) or 1.0 l/min, and air which had been filtered by the fabric was sucked into the dust counter and the amount (n) of dust having a size of 0.3 μm or more was counted. The amount (n<sub>0</sub>) of dust having a size of 0.3 μm or more at room temperature had been separately counted. The dust-collecting

efficiency was calculated according to the following equation (2):

$$\eta = (n_0 - n) / n_0 \quad (2)$$

At the time of measurement of  $n$ , the pressure in the funnel (at a place close to the fabric surface) is simultaneously measured by a manometer, and the difference (pressure drop,  $\text{mmH}_2\text{O}$ ) between the measured pressure and the atmospheric pressure was determined. The lower the air permeability of the fabric, the higher the pressure loss. Accordingly, if the filtration rate was constant, the pressure loss corresponded to the air permeability of the fabric. When the air suction rate in the counter was adjusted to  $0.3 \mu/\text{min}$  or  $1.0 \text{l}/\text{min}$ , the filtration rate was  $0.02 \text{ cm/sec}$  or  $0.066 \text{ cm/sec}$ . When the difference in pressure between the space between the dust-free clothing and the undergarment at the time of actual working on wearing of the dust-free clothing and the space outside the dust-free clothing was measured in advance by the above-mentioned manometer, it was found that this pressure difference was smaller than  $0.4 \text{ mmH}_2\text{O}$ .

(3) Air permeability

The air permeability was determined according to the Fazir method of JIS L-1096.

(4) Moisture permeability

The moisture permeability was determined according to the cup method of JIS L-0208 (at a temperature of  $40^\circ \text{C}$ . and a relative humidity of 90%).

(5) Dust-preventive effect of dust-free clothing

A box having an inner capacity of  $0.7 \text{ m}^3$  having an air inlet arranged in the ceiling portion and an air outlet arranged at a lower part of the side wall was placed in a clean bench having a cleanliness of class 100 or less. A person wearing dust-free clothing enters into this box and the quantity of dust generated due to the motions of the person was measured by the above-mentioned dust counter. The air cleanliness, (hereinafter referred to as "B/G") of the box before entrance of the person is substantially equal to that in the clean bench containing 3 to 4 dusts having a size of  $0.3 \mu\text{m}$  or more per liter. The person wore a commercially available cotton shirt below the dust-free clothing and also wore boots, a hood, and gloves for a dust-proof room. The dust-free clothing, boots, and other goods used were anti-electrostatic articles made by using electrically conductive yarns. The motions of the person conducted in the box were stamping and hand swinging (both the feet are kept on the ground). The frequency of each motion was 90 times per minutes. Dust generated by the motions of the person in the box flowed out from the air outlet together with an air current. The amount of dust was measured at the center of the air outlet and the amount of dust generated was determined by subtracting B/G from the counted number. Incidentally, when the above-mentioned stamping was carried out in the state where only the undergarments (cotton briefs and cotton long-sleeved shirt) were worn, the amount of generated dust was as large as 7160 per liter.

(6) Thickness of fabric

The thickness of a fabric was measured according to the method of JIS L-1079.

(7) Electrostatic charge density

The electrostatic charge density was determined according to the chargeability test method (Faraday gauge method) for antistatic working clothes, described in Recommended Standards of Construction of Appliances used for Protection against Electrostatic Hazards,

February, 1983, pages 154 through 161, issued by Research Institute of Industrial Safety, Japan. The test was conducted at a temperature of  $20^\circ \text{C}$ . and a relative humidity of 30%. Nylon and polyacrylonitrile fabrics were used as standard fabrics.

EXAMPLE 1

A green plain weave was produced by using, as warps, polyethylene terephthalate multi-filament yarns having a yarn count of 75 de/72 fil and a twist number of 250 T/M and doubled yarns formed by doubling and twisting, at a twist number of 250 T/M the above-mentioned yarns and electroconductive yarns (Trademark: Metalian, supplied by Teijin Limited) having, denier of 22 and an electric resistivity of  $8 \times 10^5 \Omega/\text{cm}$  and, as weft untwisted polyethylene terephthalate multi-filament yarns having a yarn count of 64 de/144 fil. In this fabric, the doubled yarns of the polyethylene terephthalate multi-filament yarn and the electrically conductive filament yarn were incorporated into the warps at intervals of 0.6 cm. The fabric was desized, scoured, and dried and was then preset at  $180^\circ \text{C}$ . The fabric was subjected to dyeing procedures with 2% owf of a fluorescent brightening agent (Trademark: Mikawhite ATN made by Nippon Kayaku K. K.) (2% owf) by using a rapid circulator dyeing machine at a temperature of  $135^\circ \text{C}$ . The dyed fabric was dried and finally heat-set at  $170^\circ \text{C}$ . Then, the fabric was calendered with a hot roll at a temperature of  $170^\circ \text{C}$ , under a linear pressure of  $30 \text{ kg/cm}^2$  at a fabric speed of 15 m/min and was then subjected to a cam-fit treatment at a temperature of  $100^\circ \text{C}$ . at a fabric speed of 20 m/min to produce a fabric usable for dust-free clothing. The properties of the resultant fabric are shown in Table 1, the volume fractions relative to various sizes of pores are shown in Table 2, the pore size distribution is shown in FIG. 2, and the dust-filtering property of the fabric is shown in Table 3. The dust-preventive property of an overall type dust-free clothing formed by using this fabric is shown in Table 4. The electrostatic charge density of the fabric is shown in Table 5.

EXAMPLE 2

A fabric for dust-free clothing was prepared in the same manner as described in Example 1 except that the warps consisted of false-twisted polyethylene terephthalate multi-filament yarns having a yarn count of 75 de/72 fil and having a twist number of 250 T/M, and doubled yarns formed by doubling and twisting, at a twist number of 250 T/M the above-mentioned yarns and the Metalian yarns and the wefts consisted of false-twisted, untwisted polyethylene terephthalate multifilament yarns having a yarn count of 75 de/72 fil. The properties of the resultant fabric are shown in Tables 1, 2, 3, and 5 and in FIG. 2.

EXAMPLE 3

A fabric for dust-free clothing was produced in the same manner as described in Example 1, except that the weave structure was changed to a  $\frac{1}{2}$  twill structure. The properties of the resultant fabric are shown in Tables 1, 2, and 3 and FIG. 3.

EXAMPLE 4

A fabric for dust-free clothing was produced in the same manner as described in Example 2, except that the twill weave structure and the densities of warps and

wefts were changed to as shown in Table 1. The properties of the resultant fabric are shown in Tables 1, to 5 and in FIG. 2.

#### EXAMPLE 5

A fabric for dust-free clothing was prepared in the same manner as described in Example 1 except that the type of wefts and the densities of warps and wefts were changed to as shown in Table 1. The properties of the resultant fabric are shown in Tables 1, 2, 3 and 5 and in FIG. 2.

#### EXAMPLE 6

##### (1) Preparation of Woven Fabric

By using a polyethylene terephthalate having an intrinsic viscosity of 0.62 (as measured at 35° C. in o-chlorophenol) and a poly- $\epsilon$ -caproamide having an intrinsic viscosity of 1.30 (as measured at 35° C. in m-cresol), there was prepared hollow composite filaments in which the above-mentioned polyester and polyamide components in the number of 16 were arranged alternately and adjacently to each other in the form of annulets and were extended in the longitudinal direction of the filaments to form a tubular structure as a whole (see Japanese Unexamined Patent Publication (Kokai) No. 51-70366). In the resultant composite filament yarn, the weight ratio of the total polyamide component to the total polyester component was 1/1, and the denier of each component filament was 0.23. The thickness of the composite filament yarn was 3.7 denier. The hollow ratio, that is, the ratio of the volume of the hollow portion to the sum of the entire volumes of the polyamide components, the polyester component, and the hollow portion was 8%.

A plain weave fabric (taffeta) having a warp density of 105 yarns/inch and a weft density of 73 yarns/inch was prepared by using, as wefts, the above-mentioned composite multifilament yarns (150 denier/40 filaments, untwisted) and, as warps, polyethylene terephthalate multifilament yarns (75 denier/72 filaments, a twist number of 300 T/M) and a doubled yarn formed by doubling and twisting, at a twist number of 200 T/M, the abovementioned polyethylene terephthalate multifilament yarns and copper iodide-containing polyethylene terephthalate monofilament yarns having an electric resistance of  $2 \times 10^8 \Omega/\text{cm}$  (supplied by Teijin Limited) and a denier of 22. The intervals of the electrically conductive yarns was 0.8 cm.

##### (2) Processing of Woven fabric

The resultant woven fabric was subjected to a wet heat treatment at 90° C. for 20 minutes in a treating bath containing 1 g/l of soda ash and 1 g/l of a detergent (Trademark: Scourol 400, made by Kao-Atlas) by using a circular dyeing machine (made by Hisaka Seisakusho K. K.). Then, the fabric was treated in the rope-like form at 30° C. for 30 minutes with a 1% emulsion of a treating agent (Trademark: Tetrosin OE-N, made by Yamakawa Yakuhin K. K. and containing 36% of o-phenylphenol) by using the circular dyeing machine (the liquor ratio was 1/30).

Then, the woven fabric was scoured at 90° C. for 20 minutes in a scouring bath containing 5 g/l of soda ash and 1 g/l of Scourol 400, heat-set at 170° C. for 30 seconds, and dyed at 130° C. for 60 minutes in an aqueous dyeing bath containing 4% a disperse dye (C.I. 63305, Trademark: Duranol Blue G made by ICI), 0.2 ml/l of acetic acid, and 1 g/l of a dispersant composed mainly of a condensation product of naphthalene-sul-

fonic acid with formamide. Then, the dyed fabric was subjected to a soaping procedure with an aqueous solution of a non-ionic detergent at 80° C. for 20 minutes and dried at 120° C. for 3 minutes.

Then, the fabric was calendered at 170° C. under a pressure of 20 kg/cm<sup>2</sup> by using a hot roll. The properties of the resultant fabric are shown in Tables 1, 2, 3, and 5 and FIG. 1. In the resultant fabric, the interval of the electrically conductive filament yarns was 0.6 cm.

#### COMPARATIVE EXAMPLE 1

A green 2/1 twill fabric was produced by using, as warps, polyethylene terephthalate multifilament yarns having a yarn count of 75 de/36 fil and a twist number of 154 T/M and doubled yarns formed by doubling and twisting, at a twist number of 200 T/M, the above-mentioned multifilament yarns, and carbon-type electroconductive filament yarns (Trademark: Metalian made by Teijin Limited) having a denier of 22 and an electric resistance of  $8 \times 10^5 \Omega/\text{cm}$  and, as wefts, false-twisted, untwisted polyethylene terephthalate multifilament yarns having a yarn count of 100 de/24 fil. In this fabric, the doubled yarns composed of the polyethylene terephthalate yarns and the electroconductive yarns were incorporated at intervals of 2 cm into the warps. The fabric was desized, scoured, and dried and was then preheat-set at 200° C. The fabric was subjected to a fluorescent brightening process with 2% owf of a brightening agent (Trademark: Mikawhite ATN (made by Nippon Kayaku K. K.) by using a liquid flow dyeing machine at 130° C. The dyed fabric was dried and finally heat-set at 180° C. to obtain a fabric usable for dust-free clothing. The properties of the fabric are shown in Tables 1 to 4 and FIG. 1.

#### COMPARATIVE EXAMPLE 2

A fabric for dust-free clothing was prepared in the same manner as described in Comparative Example 1 except that the polyethylene terephthalate filaments had a triangular cross-sectional profile and a yarn count of 100 de/48 fil were used as the warps, polyethylene terephthalate multifilament yarns having a triangular cross-sectional profile and a yarn count of 100 de/48 fil were used as the wefts, and the weave structure was changed to a plain weave. The properties of the resultant fabric are shown in Tables 1 to 4 and FIG. 1.

#### COMPARATIVE EXAMPLE 3

A piece for a clothing was cut out from a commercially available dust-proof fabric. This fabric had a 3/2 twill structure in which polyester multifilament yarns of 82 de/36 fil were used as warps at a density of 160 yarns/inch and polyester multifilament yarns of 83 de/72 fil as wefts at a density of 127 yarns/inch. Electrically conductive filament yarns were incorporated into the warps at an interval of 0.45 cm. The surface of this woven fabric was coated with a water-proof moisture-permeable resin in a thickness of about 15  $\mu\text{m}$ . The weight of this fabric was 118 g/m<sup>2</sup> and the thickness of the fabric was 0.115 mm. The fabric had an air permeability of 0.2 cc/cm<sup>2</sup>/sec and a moisutre permeability of 3000 g/m<sup>2</sup>/24 hours. Both the air permeability and the moisture permeability of the fabric were unsatisfactory. The properties of the fabric are shown in Tables 1, 3, and 4.

## COMPARATIVE EXAMPLE 4

A composite fabric was prepared by laminating a water-proof, moisture-permeable polyurethane resin film on the back surface of the fabric prepared in Example 1. The properties of the resultant composite fabric are shown in Tables 1 to 4.

## COMPARATIVE EXAMPLE 5

A green 2/2 twill weave fabric was prepared by using, as warps, polyethylene terephthalate multifilament yarns having a yarn count of 100 de/48 fil and twist number of 250 T/M and doubled yarns formed by doubling and twisting at a twist number of 250 T/M, the above-mentioned polyethylene terephthalate multifilament yarns and the electrically conductive carbon filament yarns and, as wefts, polyethylene terephthalate multi-filament yarns having a yarn count of 75 de/36 fil. The fabric was processed in the same manner as described in Comparative Example 2. The properties of the resultant fabric for dust-free clothing are shown in Tables 1 to 3 and FIG. 3.

## COMPARATIVE EXAMPLE 6

A piece of fabric was cut out from a commercially available dust-proof fabric. This fabric had a herring-bone twill structure and comprised polyethylene terephthalate multifilament yarns as the warps and wefts. In this fabric, no electrically conductive filament yarn was used. The air permeability of the fabric was 3.7 cc/cm<sup>2</sup>/sec. The properties of this fabric are shown in Tables 3 and 5.

## COMPARATIVE EXAMPLE 7

A piece of fabric was cut out from a commercially available dust-proof fabric. The fabric was a plain weave fabric comprised polyethylene terephthalate multifilament yarns as both the warps and wefts. The electrically conductive filament yarns were incorporated into the warps at intervals of 1 cm. The air permeability of the fabric was 12.1 cc/cm<sup>2</sup>/sec. The dust-filtering property of the fabric is shown in Table 3. It was confirmed with the naked eye that the cavities in the weave texture were as large as in the fabric of Comparative Example 1, even if the pore diameter distribution was not measured.

## COMPARATIVE EXAMPLE 8

A piece of fabric was taken out from a commercially available dust-proof fabric. This fabric had a 2/1 twill structure composed of polyethylene terephthalate multifilament yarns as both the warps and wefts, and the electrically conductive filament yarns were incorporated at an interval of 1 cm into the warps. The air permeability of the fabric was 13.0 cc/cm<sup>2</sup>/sec. It was observed with the naked eye that the pores formed in the weave structure were as large as in the fabric of Comparative Example 1, even if the pore size distribution was not measured.

## COMPARATIVE EXAMPLE 9

A piece of fabric was cut out from a commercially available dust-proof fabric. The fabric had a 2/2 twill weave structure comprising, as the warps, polyethylene terephthalate multifilament yarns having a yarn count of 162 de/48 fil at a density of 128 yarns/inch and, as the wefts, polyethylene terephthalate multifilament yarns having a yarn count of 65 de/36 fil at a density of 110

yarns/inch, and the electrically conductive filament yarns were incorporated at intervals of 1.3 cm into the warps. The air permeability of the fabric was 1.7 cc/cm<sup>2</sup>/sec. The dust-filtering property of the cut-out fabric is shown in Table 3. It was confirmed with the naked eye that the pores in the weave structure were as large as in the fabric described in Comparative Example 2.

## COMPARATIVE EXAMPLE 10

A piece of fabric was cut out from a commercially available dust-proof fabric. This fabric had a 1/3 twill weave structure comprising, as the warps, polyethylene terephthalate multifilament yarns having a yarn count of 100 de/48 fil at a density of 125 yarns/inch and, as the wefts, polyethylene terephthalate multifilament yarns having a yarn count of 100 de/48 fil at a density of 99 yarns/inch, and the electrically conductive filament yarns were incorporated at intervals of 0.6 cm into the warps. The air permeability of the fabric was 17.1 cc/cm<sup>2</sup>/sec. The dust-filtering property of the cut-out fabric is shown in Table 3. It was confirmed with the naked eye that the pores in the weave structure were as large as in the fabric of Comparative Example 1, even if the pore size distribution of the fabric was not measured.

## COMPARATIVE EXAMPLE 11

The back surface of a Nylon 6 fabric comprising, as warps, Nylon 6 multifilament yarns having a yarn count of 120 de/24 fil at a density of 144 yarns/inch and, as wefts, nylon 6 multifilament yarns having a yarn count of 120 de/24 fil at a density of 88 yarns/inch was coated with 4%, based on the weight of the fabric, of an acrylic resin. The weight of the treated fabric was 115 g/m<sup>2</sup>, the thickness was 0.177 mm, and the air permeability was 0.37 cc/cm<sup>2</sup>/sec. The dust-filtering property of the treated fabric is shown in Table 3. Though the air permeability of the fabric was poor, the dust-collecting property of the fabric was unsatisfactory. It is apparent that even if pores in the woven structure are filled with a resin to reduce the air permeability, the dust-collecting property is not so improved.

## EXAMPLE 7

The fabric as described in Example 4 was calendered at a hot roll temperature of 180° C. under a linear pressure of 30 kg/cm at a roll speed of 0.5 m/min. The moisture permeability of the resultant fabric was 6000 g/m<sup>2</sup>/24 hours, and the air permeability was 0.9 cc/cm<sup>2</sup>/sec. The integrated volumes of the pores relative to the pore size are shown in Table 2, the pore size distribution is shown in FIG. 3, and the dust-collecting efficiency is shown in Table 4.

## EXAMPLE 8

A plain weave fabric was prepared by using, as wefts, the same hollow composite multifilament yarns (150 denier/40 filaments, untwisted) as used in Example 1 and doubled yarns each formed by doubling and twisting, at a twist number of 200 T/M, the above-mentioned composite multifilament yarn and a copper iodide-containing, electrically conductive polyethylene terephthalate monofilament yarn having a denier of 22 and, as warps, polyethylene terephthalate multifilament yarns (75 denier/72 filaments, twisted at a twist number of 300 T/M) and doubled yarns each formed by doubling and twisting, at a twist number of 200 T/M, the

above-mentioned polyethylene terephthalate multifilament yarn and the above-mentioned copper iodide-con-

were not incorporated. The frictional charge density of the fabric is shown in Table 5.

TABLE 1

| Example No.              | Structure<br>(de/fil of warp ×<br>de/fil of weft)   | Type            | Properties of Fabrics |                      |                               | Thickness<br>(mm) | Moisture<br>Permeability<br>(g/m <sup>2</sup> /24 hours) | Air<br>Permeability<br>(cc/cm <sup>2</sup> /min) |
|--------------------------|-----------------------------------------------------|-----------------|-----------------------|----------------------|-------------------------------|-------------------|----------------------------------------------------------|--------------------------------------------------|
|                          |                                                     |                 | Warp<br>(yarns/inch)  | Weft<br>(yarns/inch) | Weight<br>(g/m <sup>2</sup> ) |                   |                                                          |                                                  |
| Example 1                | T75/72 × T64/144                                    | plain weave     | 163                   | 106                  | 92                            | 0.100             | 7400                                                     | 1.4                                              |
| Example 2                | TW75/72 × TW75/72                                   | "               | 155                   | 94                   | 94                            | 0.111             | 7800                                                     | 2.2                                              |
| Example 3                | T75/22 × T64/144                                    | 2/1 twill weave | 214                   | 116                  | 124                           | 0.130             | 7400                                                     | 3.8                                              |
| Example 4                | TW75/72 × TW75/72                                   | "               | 215                   | 114                  | 129                           | 0.151             | 7500                                                     | 7.2                                              |
| Example 5                | T75/72 × T75/72                                     | plain weave     | 169                   | 108                  | 107                           | 0.105             | 6800                                                     | 0.7                                              |
| Example 6                | T75/72 × TN150/40<br>(splitted to 16<br>components) | "               | 148                   | 85                   | 133                           | 0.149             | 7000                                                     | 0.7                                              |
| Comparative<br>Example 1 | T75/36 × TW100/24                                   | 2/1 twill weave | 186                   | 95                   | 108                           | 0.133             | 7100                                                     | 15.0                                             |
| Comparative<br>Example 2 | TΔ100/48 × TΔ100/48                                 | plain weave     | 102                   | 70                   | 99                            | 0.130             | 7300                                                     | 3.0                                              |
| Comparative<br>Example 3 | resin-laminated<br>fabric                           | —               | 160                   | 127                  | 118                           | 0.115             | 3000                                                     | 0.26                                             |
| Comparative<br>Example 4 | resin-laminated<br>fabric                           | —               | 163                   | 106                  | 113                           | 0.170             | 2000                                                     | below 0.2                                        |
| Comparative<br>Example 5 | T100/48 × T75/36                                    | 2/2 twill weave | 170                   | 107                  | 125                           | 0.138             | 7500                                                     | 2.5                                              |

taining, electrically conductive polyethylene terephthalate monofilament yarn. In this fabric, the warp density was 105 yarns/inch and the weft density was 73 30 yarns/inch, and the electrically conductive polyethylene terephthalate monofilament yarns were incorporated at intervals of 0.8 cm into both the warps and wefts in a lattice pattern.

The same treatments as described in Example 1 were 35 applied to the fabric. A dust-proof fabric in which the electrically conductive polyethylene terephthalate monofilament yarns were arranged in a lattice pattern at intervals of 0.6 cm was obtained.

#### EXAMPLE 9

A green plain weave fabric was prepared by using, as warps, polyethylene terephthalate multifilament yarns having a yarn count of 75 de/72 fil and a twist number of 250 T/M, and doubled yarns each formed by doubling and twisting, at a twist number of 250 T/M, the above-mentioned polyethylene terephthalate multifilament yarns and the electrically conductive carbon filament yarns (Metalian) having a denier of 22 and, as wefts, untwisted polyethylene terephthalate multifilament yarns having a yarn count of 64 de/144 fil yarns and doubled yarns each formed by doubling and twisting, at a twist number of 250 T/M, the above-mentioned polyethylene terephthalate multifilament yarn and the electrically conductive carbon filament yarn. The doubled yarns of the polyethylene terephthalate multifilament yarn and the electrically conductive carbon filament yarn were incorporated at intervals of 0.6 cm into both the warps and wefts. The same treatments as described in Example 1 were applied to the fabric. A 55 fabric useful for dust-free clothing was obtained. The frictional charge density of this fabric is shown in Table 5.

#### COMPARATIVE EXAMPLE 12

A comparative fabric was prepared in the same manner as described in Example 1, except that the electrically conductive carbon filament yarns, (Metalian)

In Table 1, the abbreviations have the following meanings.

T: polyethylene terephthalate (PET) multifilament yarn  
TN: PET and Nylon 6 hollow composite filament yarn, described in Example 6

W: false-twisted textured bulky yarn

de: denier

fil: the number of individual filaments

A: triangular cross-sectional profile (unless especially indicated, the cross-sectional profile is circular).

TABLE 2

| Example No. | Entire integrated volume of all pores (ml/g) | % based on entire integrated volume |                |                 |
|-------------|----------------------------------------------|-------------------------------------|----------------|-----------------|
|             |                                              | 0.9 μm-9.9 μm                       | 9.9 μm or more | 42.6 μm or more |
| Example 1   | 0.5120                                       | 33.1                                | 53.0           | 15.4            |
| Example 2   | 0.5717                                       | 30.9                                | 30.9           | 18.4            |
| Example 3   | 0.4333                                       | 43.4                                | 38.9           | 14.6            |
| Example 4   | 0.6822                                       | 39.5                                | 50.0           | 14.0            |
| Example 5   | 0.5667                                       | 28.7                                | 55.5           | 20.6            |
| Example 6   | 0.5337                                       | 48.5                                | 33.8           | 7.7             |
| Example 7   | 0.4783                                       | 33.3                                | 49.9           | 14.5            |
| Comparative | 0.5977                                       | 17.2                                | 71.1           | 51.0            |
| Example 1   |                                              |                                     |                |                 |
| Comparative | 0.7422                                       | 13.6                                | 76.6           | 43.1            |
| Example 2   |                                              |                                     |                |                 |
| Comparative | 0.5480                                       | 24.0                                | 63.0           | 45.2            |
| Example 3   |                                              |                                     |                |                 |

TABLE 3

| Example No. | Dust-Filtering Property            |              |                                         |              |
|-------------|------------------------------------|--------------|-----------------------------------------|--------------|
|             | Filtration speed (V <sub>0</sub> ) |              |                                         |              |
|             | Dust-collecting efficiency (η)     |              | Pressure loss (ΔP (mmH <sub>2</sub> O)) |              |
| Example No. | 0.020 cm/sec                       | 0.066 cm/sec | 0.020 cm/sec                            | 0.066 cm/sec |
| Example 1   | 0.87                               | 0.78         | 0.6                                     | 2.0          |
| Example 2   | 0.90                               | 0.80         | 0.2                                     | 0.7          |
| Example 3   | 0.87                               | 0.78         | 0.1                                     | 0.4          |
| Example 4   | 0.89                               | 0.79         | 0.1                                     | 0.2          |
| Example 5   | 0.96                               | 0.93         | 1.0                                     | 3.2          |
| Example 6   | 0.996                              | 0.98         | 0.6                                     | 2.6          |
| Example 7   | 0.90                               | 0.79         | 0.5                                     | 1.4          |
| Comparative | 0.65                               | 0.45         | 0.0                                     | 0.1          |

TABLE 3-continued

| Example No. | Dust-Filtering Property               |              |              |                                                  |
|-------------|---------------------------------------|--------------|--------------|--------------------------------------------------|
|             | Filtration speed ( $V_p$ )            |              |              |                                                  |
|             | Dust-collecting efficiency ( $\eta$ ) | 0.020 cm/sec | 0.066 cm/sec | Pressure loss ( $\Delta P$ (mmH <sub>2</sub> O)) |
| Example 1   | 0.75                                  | 0.63         | 0.0          | 0.2                                              |
| Comparative | *                                     | *            | *            | *                                                |
| Example 2   | *                                     | *            | *            | *                                                |
| Comparative | *                                     | *            | *            | *                                                |
| Example 3   | *                                     | *            | *            | *                                                |
| Comparative | 0.70                                  | 0.65         | 0.0          | 0.2                                              |
| Example 4   | 0.50                                  | 0.42         | 0.0          | 0.1                                              |
| Comparative | 0.48                                  | 0.38         | 0.0          | 0.1                                              |
| Example 5   | 0.51                                  | 0.31         | 0.0          | 0.1                                              |
| Comparative | 0.65                                  | 0.58         | 0.0          | 0.2                                              |
| Example 6   | 0.56                                  | 0.48         | 0.0          | 0.1                                              |
| Comparative | 0.55                                  | 0.54         | 16.6         | 70.0                                             |
| Example 11  |                                       |              |              |                                                  |

Note:

\*Since the air permeability is extremely low, the pressure loss  $\Delta P$  is extremely increased at the measurement of the dust-collecting efficiency ( $\eta$ ). As result, leakage of the dust from the seal is caused and the dust-collecting efficiency ( $\eta$ ) cannot be measured.

TABLE 4

| Example No. | Dust-Preventive Property of Dust-Proof Clothing                              |               |          |
|-------------|------------------------------------------------------------------------------|---------------|----------|
|             | Number (dusts/1) of generated dusts having size of 0.3 $\mu\text{m}$ or more |               |          |
|             | Motions                                                                      | Hand swinging | Stamping |
| Example 1   | 26                                                                           | 34            | 30       |
| Example 4   | 45                                                                           | 43            | 33       |
| Example 6   | 5                                                                            | 7             | 11       |
| Comparative | 125                                                                          | —             | 61       |
| Example 1   | 69                                                                           | 61            | 30       |
| Comparative | 111                                                                          | 19            | 60       |
| Example 2   | 36                                                                           | 16            | 37       |
| Comparative |                                                                              |               |          |
| Example 4   |                                                                              |               |          |

TABLE 5

| Example No.            | Electrostatic charge density* |  |
|------------------------|-------------------------------|--|
|                        | ( $\mu\text{C}/\text{m}^2$ )  |  |
| Example 1              | 3.8                           |  |
| Example 2              | 3.7                           |  |
| Example 3              | 3.7                           |  |
| Example 4              | 4.0                           |  |
| Example 5              | 3.5                           |  |
| Example 6              | 3.3                           |  |
| Example 8              | 2.7                           |  |
| Example 9              | 1.9                           |  |
| Comparative Example 6  | 14.6                          |  |
| Comparative Example 12 | 15.1                          |  |

Note

\*The density of the electrostatic charge was measured 5 times by rubbing the fabric with each of Nylon 6 and acrylic fabrics. The mean value is calculated, and the largest value between the mean value obtained with respect to the nylon fabric and the mean value obtained with respect to the acrylic fabric was indicated in the table.

From Table 2 and FIGS. 1 through 3 showing the relationship between the volume fraction of pores and the size of the pores in a fabric, it is understood that in each of the fabrics of the comparative examples, the size of the pores having a maximum volume fraction was 50

to 60  $\mu\text{m}$  or larger and the volume fraction proportion of pores having a size of 42.6  $\mu\text{m}$  or more is very large, while the integrated volume proportion of pores having a size in a range of from 0.1  $\mu\text{m}$  to 9.9  $\mu\text{m}$  is very small. 5 In contrast, in each of the fabrics of the examples in accordance with the present invention, the size of pores having a largest integrated volume proportion is smaller than that in the comparative examples, and the integrated volume proportion of pores having a size of 42.6  $\mu\text{m}$  or more is drastically reduced and the integrated volume proportion of pores having a size in a range of from 0.1  $\mu\text{m}$  to 9.9  $\mu\text{m}$  is increased. Namely, in each of the fabrics of the comparative examples, the volume of the inter-filament bundle pores is large and the volume of the inter-filament pores is small. On the other hand, in each of the fabrics of the examples, the volume of the inter-filament bundle pores is drastically reduced and the volume of the inter-filament pores is increased. This characteristic is especially prominent in the fabric of Example 6. In short, the fabrics of the present invention have a structure having a higher dust-filtering property than the fabrics of the comparative examples.

With respect to the above-mentioned fabrics, the dust-collecting efficiency ( $\eta$ ) and the pressure loss ( $\Delta P$ ) were measured. The results are shown in Table 3. In the conventional fabrics for dust-free clothing, shown in Comparative Examples 1, 2, and 4 through 12, the value ( $\eta$ ) is 0.75 at highest and is ordinarily in a range of from about 0.5 to about 0.6. In case of the conventional fabrics of Comparative Examples 3 and 4, the air permeability is so poor that the value ( $\eta$ ) cannot be determined because of too high a pressure loss, and these fabrics are not suitable for making dust-free clothing. Furthermore, from the results of Comparative Example 11, it is seen that even if in order to reduce the air permeability, a coating resin is applied to a woven fabric and pores in the fabric are filled with the resin, a fabric having a high dust-collecting efficiency cannot be obtained. In contrast, in the fabrics of the examples in accordance with the present invention, the dust-collecting efficiency is about 0.9 or higher. It is seen that the fabrics of the present invention are improved over the fabrics of the comparative examples in the dust-collecting efficiency. 35 The dust-collecting efficiency of the fabric of Example 6 is especially high and about 1.00, and this fabric can collect substantially 100% of dust while allowing permeation of air. When the fabric of Example 5 is compared with the fabric of Example 6, it is seen that although the fabric of Example 6 has a lower pressure loss and a slightly lower air permeability, this fabric has a higher dust-collecting efficiency. It is considered that this is due to the fact that the integrated volume of the inter-filament pores in the fabric of Example 6 is large. 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790

of 0.1 to 9.9  $\mu\text{m}$  is large, the dust-collecting efficiency of the fabric becomes high, and it is seen that there is established a close interrelation between the pore characteristic (structure) and the dust-collecting efficiency of the fabric.

Overall type dust-free clothing were prepared by using the fabrics shown in Table 4. The dust-proof properties of these dust-free clothing were examined by checking the generation of dust caused when this clothing were actually worn. When hand swinging and stamping motions were carried out, in case of the dust-free clothing of Examples 1, 4, and 6 and Comparative Examples 1 through 4, the amount of generated dust tended to decrease with reduction of the air permeability of the fabric. However, when the dust-free clothing of Comparative Examples 3 and 4 composed of a fabric having no substantial air permeability were worn, the amount of generated dust was increased on the contrary. When openings in the sleeve edges (both hands and both feet) and the neck portion of the dust-free clothing were sealed with a view to clarifying the cause of the above phenomenon and so as to prevent the discharge of the dust from these openings, the amount of generated dust was drastically reduced. Namely, in the dust-free clothing of Comparative Examples 3 and 4, since they had no air permeability, discharge of air caused by the motions was effected only through the openings in the sleeve edges and neck portion, and contaminated air was discharged outside directly through these openings.

From the foregoing results, it is clear that the fabric of the present invention having a certain air permeability and a high dust-filtering property is suitable as a fabric for making dust-free clothing. Since the fabrics of the comparative examples have a low dust-filtering property or too high or too low an air permeability, clothing made of these fabrics exhibits a poor dust-preventive property. Generation of dust from the dust-free clothing of Example 6 is very small. That is, the fabric of Example 6 is especially excellent as a fabric for making dust-free clothing. Moreover, although the fabric of Example 4 has a high air permeability, generation of dust from the dust-free clothing made of this fabric is small.

When generation of dust was examined, the comfort was simultaneously evaluated with respect to each dust-free clothing. With respect to each clothing, the same person dressed up for an operation in a clean room according to customary wearing procedures and performed the stamping motion for 6 minutes. The comfort was checked. The sweating state of the person after the stamping motion was such that the skin was slightly wet with sweat. From the test results, it was found that as the air permeability of the fabric of the dust-free clothing is lower, the uncomfortable feeling becomes stronger. In the dust-free clothing of Comparative Examples 1 and 2 and Examples 1, 4, and 6, there was no uncomfortable feeling at all or there was no substantial uncomfortable feeling. However, in the dust-free clothing of Comparative Examples 3 and 4, the uncomfortable feeling was extremely prominent and the sweating skin adhered stickily to the fabric, i.e., the comfort was poor. It is considered that the reason is that the fabrics of Comparative Examples 3 and 4 were insufficient in air permeability and moisture permeability.

In view of the quantities of electrostatic charge shown in Table 5, it is clear that in the fabrics of the

comparative examples comprising no electrically conductive yarn, the quantities of the electrostatic charge are large and the antistatic property is insufficient, while in the fabrics of the examples in accordance with the present invention, the quantities of the electrostatic charge are small, that is, less than 7  $\mu\text{C}/\text{m}^2$ , and the antistatic property is excellent. The fabric of Example 8 comprising electrically conductive yarns in both the warps and wefts had an especially high antistatic effect.

We claim:

1. A dust-proof fabric comprising a plurality of filament yarns having a denier of from 20 to 400 and consisting of a plurality of individual filaments having a denier of 3.5 or less, which fabric has a number of pores formed therein and exhibits an air permeability of from 0.3 to 10  $\text{ml}/\text{cm}^2/\text{sec}$  and, in which fabric, the integrated volume proportion of the pores having a size of 43  $\mu\text{m}$  or more corresponds to 40% or less of the entire integrated volume of all the pores.
2. The dust-proof fabric as claimed in claim 1, wherein the integrated volume proportion of the pores having a size of 43  $\mu\text{m}$  or more is 25% or less based on the entire integrated volume of all the pores.
3. The dust-proof fabric as claimed in claim 1, wherein the integrated volume proportion of the pores having a size of from 0.1  $\mu\text{m}$  to 10  $\mu\text{m}$  corresponds to 28% or more of the entire integrated volume of all the pores.
4. The dust-proof fabric as claimed in claim 3, wherein the integrated volume proportion of the pores having a size of from 0.1  $\mu\text{m}$  to 10  $\mu\text{m}$  corresponds to 40% or more of the entire integrated volume of all the pores.
5. The dust-proof fabric as claimed in claim 1, which is in the form of a woven fabric composed of a plurality of warps and wefts consisting of the filament yarns.
6. The dust-proof fabric as claimed in claim 5, wherein the warps and/or wefts contain electrically conductive filament yarns having an electric resistivity of  $10^{10} \Omega/\text{cm}$  or less and arranged at intervals of from 3 mm to 50 mm.
7. The dust-proof fabric as claimed in claim 1, which fabric has a thickness of from 0.05 mm to 0.40 mm.
8. The dust-proof fabric as claimed in claim 1 or 5, wherein the denier of the individual filaments is 1.5 or less.
9. The dust-proof fabric as claimed in claim 8, wherein the denier of the individual filaments is 0.5 or less.
10. The dust-proof fabric as claimed in claim 1, wherein the individual filaments are selected from the group consisting of polyester filaments, polyamide filaments, polyaramide filaments, polyolefin filaments, polyvinyl polymer filaments, rayon filaments, cellulose acetate filaments, silk filaments, and glass filaments.
11. The dust-proof fabric as claimed in claim 9, wherein the individual filaments having a denier of 0.5 or less are ones prepared from peel-separating composite filaments composed of a polyester filamentary constituent and a polyamide filamentary constituent connected to each other by peel-separating the polyester and polyamide filamentary constituents from each other.
12. The dust-proof fabric as claimed in claim 1, wherein at least a portion of the filament yarns comprises bulky multifilament yarns.

\* \* \* \* \*